

Oct. 31, 1939.

L. A. CLARKE

2,178,321

SOLVENT REFINING

Filed April 2, 1937



LOUIS A. CLARKE  
INVENTOR

BY *P. J. Nealon*

ATTORNEY

## UNITED STATES PATENT OFFICE

2,178,321

## SOLVENT REFINING

Louis A. Clarke, Fishkill, N. Y., assignor to The Texas Company, New York, N. Y., a corporation of Delaware

Application April 2, 1937, Serial No. 134,465

2 Claims. (Cl. 196—13)

This invention relates to refining hydrocarbon oil by solvent extraction.

The invention contemplates a method of refining lubricating oil stocks of different characteristics by solvent extraction in a related operation for the production of lubricating oil products of desired characteristics. The invention has reference to the solvent extraction of lubricating oil fractions derived from different crude sources, and particularly the extraction of a high grade and a low grade stock in a related operation.

The invention concerns, for example, the refining of residual lubricating oil fractions derived from different crude sources and by extraction with a solvent that is capable of effectively extracting asphaltic as well as low viscosity index constituents from the oil.

The method of my invention involves subjecting a high grade lubricating oil stock to extraction in a primary stage to produce a raffinate phase comprising oil of quite high viscosity index and an extract phase containing oil of lower viscosity index. These phases are separately withdrawn and the extract phase is subjected to a further extraction in a secondary extraction stage along with a lower grade of lubricating oil stock. Secondary raffinate and extract phases are produced in this secondary stage, and the secondary raffinate phase so produced comprises oil of relatively high viscosity index while the secondary extract phase comprises heavy extract oil of relatively low viscosity index.

The extraction may be effected with the same type of selective solvent in both stages. By selective solvent I contemplate a solvent having selective action as between low and high viscosity index constituents of the oil, such as furfural, phenol, nitrobenzene, etc. A solvent which I have found to be particularly suitable for this purpose comprises a chlorinated phenol mixture obtained by chlorinating crude phenol.

A chlorinated phenol mixture such as I contemplate is obtained by chlorinating crude phenol under conditions such that at least 60% of the phenol is chlorinated to produce a mixture comprising mainly a mixture of ortho- and para-monochlorophenol which may contain some unreacted phenol as well as a small amount of dichlorophenol. This chlorinated mixture is treated with sufficient alkali to remove hydrogen chloride formed during the chlorination, and after removal of the hydrogen chloride the mixture is distilled to a temperature of around 220° at atmospheric pressure to remove as a dis-

tillate a mixture having the following composition:

Table 1

|                   | Per cent by volume |    |
|-------------------|--------------------|----|
| Phenol            | 5                  |    |
| Parachlorophenol  | 0-40               |    |
| Orthochlorophenol | 30-55              |    |
| Dichlorophenol    | 20-50              |    |
|                   | 0-3                | 10 |

It has been found that a solvent mixture having a composition within the range above specified is particularly suitable for the purpose of this invention. The relative proportions of ortho- and para-monochlorophenol in the mixture can be varied to some extent, but it is desirable that substantial proportions of each of these components be present and that the parachlorophenol should predominate; that is, a mixture of para- and orthomonochlorophenol containing about 50 to 75% of the para- compound provides a satisfactory mixture.

A chlorinated phenol mixture which we have found particularly effective has the following composition:

Table 2

|                   | Per cent by volume |    |
|-------------------|--------------------|----|
| Phenol            | 15                 |    |
| Orthochlorophenol | 31                 |    |
| Parachlorophenol  | 51                 | 30 |
| Dichlorophenol    | 3                  |    |

Orthochlorophenol alone has too high solubility for the constituents of lubricating oil. On the other hand, the para compound solidifies at temperatures around room temperature. A mixture of the two in the proportions above indicated possesses many advantages as a refining solvent for hydrocarbon oil which cannot be secured by the use of the isomers separately. One advantage of a chlorphenol mixture, such as above described, resides in its ability to extract resinous asphaltic constituents from the oil to a very high degree.

This type of solvent is particularly efficient in the case of residual lubricating oil stocks from the standpoint of producing lubricating oil therefrom having a relatively light color and a relatively low residual carbon content.

In order to illustrate the process of my invention as applied to the refining of residual lubricating oil stocks, reference will now be made to the accompanying drawing showing a flow diagram of the process.

A high grade residual lubricating oil fraction, 55

such as derived from Mid-Continent crude, is mixed with propane and conducted to a settler 1. The propane is mixed with the oil in the ratio of about three parts of propane to one part of 5 oil, or sufficient so as to cause precipitation of hard asphaltic constituents, and which is brought about by maintaining the mixture within the settler at a temperature of around 120° F. The hard asphaltic constituents are drawn off from the bottom of the settler, while the solution of oil in propane is drawn off from the top of the 10 settler and conducted to the lower portion of a primary extractor 2.

The primary extractor 2 may comprise a vertical column packed with suitable contacting material, such as Raschig rings, and adapted to effect countercurrent contact between oil and extraction solvent.

The extraction solvent, having the composition set forth in Table 2 above, is introduced to 20 the upper portion of the extractor 2 in the proportion of about two to four parts of solvent to one part of undiluted oil. The extractor 2 is maintained at a temperature of around 80 to 120° F. 25 The raffinate phase accumulating in the upper portion of the extractor 2 under these conditions will comprise oil of relatively high viscosity index and suitable, for example, as an airplane oil. This primary raffinate phase is withdrawn and 30 the solvent recovered therefrom.

The primary extract phase will contain oil of lower viscosity index, a substantial proportion of which is of intermediate character, as a lubricating oil product. This oil is dissolved in the main body of the extraction solvent, and by the method 35 of my invention is introduced to the mid-point of a secondary extractor 3.

Fresh chlorphenol mixture is introduced to the upper portion of this secondary extractor, while 40 a lower grade of residual lubricating oil stock is introduced to the lower portion of the extractor 3.

This lower grade stock advantageously comprises a residual lubricating oil fraction derived from a Coastal type of crude, or from a crude, 45 such as Marvel crude. This low grade residual fraction is also mixed with propane in the proportion of about five or six parts of propane to one part of oil, and the mixture introduced to a settler 4 wherein precipitation of hard asphaltic constituents is brought about.

50 The hard asphaltic matter so precipitated is withdrawn as indicated while the remaining solution of oil and propane is introduced to the lower portion of the extractor 3, as previously indicated.

55 This low grade residuum is thus brought into countercurrent contact with the extraction solvent in the presence of the primary extract phase drawn off from the primary extractor 2. The extraction solvent is introduced to the upper portion 60 of the secondary extractor 3 in the ratio of about two to four parts of solvent to one part of low grade oil introduced to the bottom of the extractor. The extraction temperature maintained within the secondary extractor 3 may be the same 65 as that maintained in the primary extractor, or, if desired, may be some lower temperature.

The secondary raffinate phase drawn off from the top of the secondary extractor 3 comprises oil of intermediate character and includes a substantial amount of the oil contained in the primary extract phase.

The secondary extract phase comprises relatively low grade oil and those asphaltic constituents particularly of a resinous character which 70 were not removed in the settlers 1 and 4.

These secondary phases are separately withdrawn and the solvent removed therefrom.

Thus, a feature of my invention involves the extraction of a low grade lubricating oil stock with a selective solvent in the presence of lubricating oil constituents extracted from a relatively high grade of lubricating oil stock.

Introduction of the primary extract phase to the secondary extraction tower permits utilizing the large amount of solvent retained in the primary extract phase as a defining agent in the secondary extraction. It also eliminates the necessity for separately stripping the solvent from the primary extract phase; that is, there is only one final extract phase produced which requires stripping to remove the solvent.

A further feature of the process resides in the flexibility of operation, permitting the obtaining of products of different characteristics.

Also, where a chlorphenol mixture of the composition disclosed is used, there is no necessity for subjecting the charge stock to a separate treatment for the removal of soft asphaltic constituents. Thus, it is unnecessary, after the hard asphaltic constituents have been removed, to subject the solution of oil in propane to different temperature conditions and different dilution ratios in order to effect removal of the soft or resinous asphaltic constituents, as would otherwise be the case. These soft asphaltic constituents are removed by the chlorphenol mixture as part of the final extract phase.

An object of the invention is to extract so-called paraffin-base or Mid-Continent oil in one stage, extract so-called naphthene-base or 3 Coastal oil in the second stage, and pass the extract from the first stage to the second stage. In this way, a specially high grade lubricating oil, such as an airplane oil, is obtained from the first stage without sacrificing yield or losing valuable lubricating oil constituents of somewhat lower grade in the extract. At the same time, a high yield of medium grade or industrial oil is obtained from the second stage, the character of this oil being superior on a yield basis to that which it is possible to obtain from a naphthene-base crude alone.

Obviously, many modifications and variations of the invention, as hereinbefore set forth, may be made without departing from the spirit and scope thereof, and therefore only such limitations should be made as are indicated in the appended claims.

I claim:

1. The method of solvent refining high grade paraffin base lubricating oil and low grade naphthene base lubricating oil derived from different crude sources comprising extracting the paraffin base lubricating oil stock with a selective solvent comprising a chlorphenol mixture containing about 15% phenol, 31% orthochlorphenol, 51% parachlorphenol, and 3% dichlorphenol, forming a primary raffinate phase comprising highly paraffinic oil and a primary extract phase rich in solvent and relatively paraffinic constituents of the oil, separating the two phases, flowing the primary extract phase through a separate extraction zone countercurrently to said naphthene base lubricating oil and in the presence of fresh solvent, forming a secondary extract phase containing low viscosity index oil, and a secondary raffinate phase comprising oil of relatively higher viscosity index, and separating the two phases.

2. The method of solvent-refining high grad

paraffin base residual lubricating oil and low grade naphthene base residual lubricating oil derived from different crude sources comprising separately deasphalting said residual lubricating oils to remove hard asphaltic constituents while retaining soft asphaltic constituents in the oil, extracting the partially deasphalting paraffin base lubricating oil with a selective solvent, forming a primary raffinate phase comprising highly paraffinic oil and a primary extract phase rich in solvent and relatively paraffinic constituents of the oil, separating the two phases, flowing the

primary extract phase through a separate extraction zone countercurrently to said naphthene base lubricating oil and in the presence of fresh solvent comprising a chlorophenol mixture containing about 15% phenol, 31% orthochlorphenol, 51% parachlorphenol, and 3% dischlorphenol, forming a secondary extract phase containing low viscosity index oil and said soft asphaltic constituents, and a secondary raffinate phase comprising oil of relatively higher viscosity index, and separating the two phases. 5 10

LOUIS A. CLARKE.